# EUROPEAN PATENT SPECIFICATION

(11) **EP 0 230 146 B1**
(45) Date of publication and mention of the grant of the patent: **06.03.1991**
(21) Application number: 86310206.7
(22) Date of filing: 30.12.1986
(51) Int. Cl.: C10G 25/00

(54) **Desulphurisation**
Entschwefelung
Désulfurisation

(30) Priority: 10.01.1986 GB 8600574
(43) Date of publication of application: 29.07.1987
(73) Proprietor: IMPERIAL CHEMICAL INDUSTRIES PLC, London SW1P 3JF (GB)
(72) Inventor: Denny, Patrick John, Croft-on-Tees§Darlington§Co Durham (GB); Carnell, Peter John Herbert, Stockton-on-Tees Cleveland (GB)
(74) Representative: Gratwick, Christopher

(56) References cited:
- US-A- 3 313 722
- US-A- 4 204 947
- US-A- 4 224 191

## Description

This invention relates to desulphurisation of feedstocks such as natural gas, or gases derived therefrom, and liquids or gases derived from oil or solid hydrocarbonaceous materials such as coal. Liquid feedstocks include LPG, naphthas, and kerosene.

Desulphurisation of such feedstocks can be effected by passing the gas through a suitable absorbent which is commonly zinc oxide and/or copper oxide and is typically in the form of granules or pellets.

When a feedstock containing absorbable sulphur compounds such as hydrogen sulphide is passed through a bed absorbent, break-through of the sulphur compounds into the effluent occurs long before the bed has reached its theoretical absorption capacity, i.e. where all of the absorbent in the bed is fully saturated, because, while the absorbent near to the bed inlet may become fully, or nearly fully, saturated with the sulphur compounds, break-through occurs well before the absorbent at the bed outlet becomes saturated.

This early break-through is particularly noticeable where the absorption temperature is low. Recently absorbents having a high surface area, typically above 20, and particularly in the range 50 to 200, m² g⁻¹ have become available and are of particular use for low temperature desulphurisation, e.g. at temperatures between -10°C and 200°C. Even so premature break-through is a problem.

We have found that the absorption capacity of a bed of a desulphurisation absorbent can usefully be increased by a temporary increase in bed temperature.

Accordingly the present invention provides a method of desulphurising a liquid or gaseous feedstock wherein the feedstock is passed through a bed of a desulphurising absorbent characterised by temporarily increasing the temperature of the absorbent bed from the normal operating temperature by at least 50°C to a temperature not in an excess of 500°C, preferably not in an excess of 400°C.

The increase in temperature is preferably to a temperature in the range 150 to 350°C and is preferably for a period of at least 1 hour. While benefits are obtained by the use of extended periods, e.g. 1 or more days, at the increased temperature, at increased temperatures above about 280°C, the higher the temperature, the shorter should be the time at that temperature, in order to avoid undue loss of surface area of the absorbent. For the aforesaid high surface area absorbents the maximum temperature is preferably below 300°C.

The maximum normal operating temperature, at which there is a noticeable benefit by temporary increase of the temperature, is about 300°C: with the aforesaid high surface area absorbents the normal operating temperature is preferably below 250°C and is preferably in the range 0 to 150°C.

The absorbent bed may be subjected to the temperature increase while on-line if the resultant increase in temperature of the desulphurised product is acceptable: however such a process also involves heating of the feedstock during at least part of the period of the increased temperature and economic considerations may render this an unacceptable mode of operation. Alternatively, and preferably, the absorbent bed is heated while the bed is off-line. Thus in a continuous process, two or more absorbent beds may be provided and while one or more beds remain on absorption duty one or more other beds are subjected to the temperature increase. Because of the heat capacity of the bed, in many cases it is not necessary to pass a fluid through the bed throughout the period for which the bed is to be subjected to an increased temperature: thus the bed may be heated via an external jacket, or by passing hot gas or liquid through the bed, until the desired maximum temperature has been achieved for a sufficient period and then the bed left static to cool down to the normal operating temperature.

In one particular form of the invention desulphurisation follows treatment of the feedstock with a molecular sieve to adsorb other impurities e.g. moisture. In such a case the molecular sieve adsorbent and the desulphurisation absorbent may be in the same vessel. Where regeneration of the molecular sieve adsorbent is effected by heating, the temporary heating of the desulphurisation absorbent may be effected at the same time as regeneration of the molecular sieve adsorbent. In a preferred form of the invention wherein a molecular sieve and an absorbent bed are employed in series, the regeneration of the molecular sieve and the temporary increase in temperature of the absorbent bed are effected by passage of a heated gas stream containing a combustible gas through the absorbent bed and through the molecular sieve. After leaving the absorbent bed and molecular sieve, the gas stream is combusted and the combustion products thereof are passed through a heat exchanger wherein heat is transferred to the gas stream employed for the regeneration step.

The time interval before the temporary heating of the desulphurisation absorbent becomes necessary will depend on the rate at which the absorbent becomes saturated, i.e. upon the absorbable sulphur compound content of the feedstock and the space velocity at which the feedstock is fed through the bed. Where the rate of sulphur pick up is very low, e.g. where the absorbable sulphur compounds content of the feedstock, and the space velocity, are low, little benefit may be obtained by the present invention. However such conditions are not normally encountered in commercial operations. The heating step should normally be effected before the sulphur break-through becomes significant.

The number of heating steps that can be employed before the bed needs recharging will depend on how saturated the bed is before each heating step and the severity, i.e. duration and temperature of the heat treatment. After a number of heat treatments, which may be as few as one, economic considerations may indicate that recharging is preferable to a further temporary temperature increase.

The sulphur compounds initially present usually include one or more of the following: H₂S, COS, and possibly CS₂, CH₃SH and others such as diethyl sulphide or tetramethylene sulphide. The total initial concentration thereof is typically in the range 1-1000 ppm v/v calculated as sulphur-equivalent H₂S. The outlet The outlet sulphur compounds concentration is typically under 1 ppm, for example under 0.5 ppm, but this is a matter of design depending on the product user's requirement.

The absorbent material preferably comprises at least 60, especially at least 80, % w/w of ZnO, calculated on its constituents non-volatile at 900°C. As used in the process, the zinc oxide may be, at least initially, wholly or partly hydrated or in the form of a salt of a weak acid. Typically the surface area of the solid material is at least 20, preferably in the range 50 to 200, m²g⁻¹; and its pore volume is typically at least 0.2. A preferred solid material for the process is characterised further by an H₂S-adsorption capacity of at least 20, especially 35-80%, of the theoretical, at temperatures up to 120°C, as determined in a standard test in which a mixture of H₂S (2000 ppm v/v), CO₂ (4% v/v) and methane (balance) is passed over the solid material as 1 bar abs. pressure and a volume hourly space velocity of 1000.

The absorbent bed can be in the form of a fixed, liftable or fluidised bed.

The invention is illustrated by the following example:

In this example the absorbent comprised a bed of 60 ml of granules (of 3-5 mm diameter) of zinc oxide of surface are a 79 m².g⁻¹ inside a tube of 25 mm internal diameter and a mixture of natural gas, to which 5% v/v of hydrogen sulphide had been added, was used as the feedstock.

The feedstock was passed through the bed at 20°C and at a space velocity of 700 hr ⁻¹ at atmospheric pressure. Break-through of H₂S occurred 93 minutes after commencing the gas flow. Calculation showed that at this stage the average sulphur content of bed was 8.6% ^{w}/w. Analysis confirmed this figure.

The gas flow was then stopped and, while still under a static atmosphere of the gas, the bed was heated to 200°C for 6 hours and then allowed to cool to 20°C.

The gas flow was recommenced: break-through occurred 29 minutes later. The calculated average sulphur content of the bed was then 11.3% w/w.

The gas flow was stopped and residual gas flushed out with nitrogen. The bed was then heated to 200°C under a static nitrogen atmosphere for 16 hours and then allowed to cool to 20°C.

The gas flow was recommenced: break-through occurred 16 minutes later. The calculated average sulphur content of the bed was then 12.8%, while analysis gave a value of 12.3% w/w.

It is seen that the two heat treatments enabled the absorption capacity of the bed to be increased by nearly 50%.

## Claims

1. A method of desulphurising a liquid or gaseous feedstock wherein the feedstock is passed through a bed of a desulphurising absorbant characterised by temporarily increasing the temperature of the absorbent bed from the normal operating temperature by at least 50°C to a temperature not in an excess of 500°C.

2. A method according to claim 1 wherein the increase in temperature is to a temperature in the range 150 to 350°C for a period of at least one hour.

3. A method according to claim 1 or claim 2 wherein the absorbent comprises zinc oxide and/or copper oxide and has a surface area above 20 m².g⁻¹, the normal operating temperature is in the range -10 to +200°C, and the maximum temperature is below 300°C.

4. A method according to any one of claims 1 to 3 wherein the absorbent comprises zinc oxide and/or copper oxide and has a surface area above 20 m².g⁻¹ and the normal operating temperature is in the range 0 to 150°C.

5. A method according to any one of claims 1 to 4 wherein at least two absorbent beds are employed and, while at least one bed is on absorption duty, at least one other of the beds is subjected to the increase in temperature and then said at least one bed that has been subjected to the temperature increase is returned to absorption duty.

6. A method according to any one of claims 1 to 5 wherein the feedstock is also treated with a molecular sieve and regeneration of the molecular sieve is effected by heating, and the regeneration of the molecular sieve is effected at the same time as the temporary increase in temperature of the absorbent bed.

7. A method according to claim 6 wherein the molecular sieve and the absorbent bed are in the same vessel.

## Patentansprüche

1. Verfahren zur Entschwefelung eines flüssigen oder gasförmigen Einsatzmaterials, bei dem das Einsatzmaterial durch ein Bett aus einem Entschwefelungs-Absorptionsmittel hindurchgehen gelassen wird, **dadurch gekennzeichnet**, daß die Temperatur des Absorptionsmittelbettes vorübergehend von der normalen Betriebstemperatur um wenigstens 50°C auf eine Temperatur von höchstens 500°C erhöht wird.

2. Verfahren nach Anspruch 1, bei dem die Temperatur für einen Zeitraum von wenigstens 1 h auf eine Temperatur im Bereich von 150 bis 350°C erhöht wird.

3. Verfahren nach Anspruch 1 oder Anspruch 2, bei dem das Absorptionsmittel Zinkoxid und/oder Kupferoxid enthält und eine spezifische Oberfläche von mehr als 20 m².g⁻¹ hat, wobei die normale Betriebstemperatur im Bereich von -10 bis +200°C und die maximale Temperatur unter 300°C liegt.

4. Verfahren nach einem der Ansprüche 1 bis 3, bei dem das Absorptionsmittel Zinkoxid und/oder Kupferoxid enthält und eine spezifische Oberfläche von mehr als 20 m².g⁻¹ hat, wobei die normale Betriebstemperatur im Bereich von 0 bis 150°C liegt.

5. Verfahren nach einem der Ansprüche 1 bis 4, bei dem wenigstens zwei Absorptionsmittelbetten eingesetzt werden und, während sich wenigstens ein Bett im Absorptionsbetrieb befindet, wenigstens ein anderes der Betten der Temperaturerhöhung unterzogen wird und dann das wenigstens eine Bett, das der Temperaturerhöhung unterzogen worden ist, in den Absorptionsbetrieb zurückgebracht wird.

6. Verfahren nach einem der Ansprüche 1 bis 5, bei dem das Einsatzmaterial auch mit einem Molekularsieb behandelt wird und das Molekularsieb durch Erhitzen regeneriert wird, wobei die Regenerierung des Molekularsiebs zu derselben Zeit wie die vorübergehende Erhöhung der Temperatur des Absorptionsmittelbettes durchgeführt wird.

7. Verfahren nach Anspruch 6, bei dem sich das Molekularsieb und das Absorptionsmittelbett in demselben Behälter befinden.

## Revendications

1. Procédé de désulfurisation d'une charge d'alimentation liquide ou gazeuse, selon lequel la charge est envoyée à travers un lit d'absorbant de désulfurisation, caractérisé en ce que la température du lit d'absorbant est augmentée temporairement d'au moins 50°C par rapport à la température normale de fonctionnement jusqu'à une température ne dépassant pas 500°C.

2. Procédé suivant la revendication 1, caractérisé en ce que l'augmentation de température va jusqu'à une température dans la gamme de 150 à 350°C pendant une période d'au moins une heure.

3. Procédé suivant la revendication 1 ou la revendication 2, caractérisé en ce que l'absorbant comprend de l'oxyde de zinc et/ou de l'oxyde de cuivre et a une aire superficielle supérieure à 20 m²g⁻¹, que la température normale de fonctionnement est dans la gamme de -10 +200°C et que la température maximum est inférieure à 300°C.

4. Procédé suivant l'une quelconque des revendications 1 à 3, caractérisé en ce que l'absorbant comprend de l'oxyde de zinc et/ou de l'oxyde de cuivre et a une aire superficielle supérieure à 20 m².g⁻¹ et que la température normale de fonctionnement est dans la gamme de 0 à 150°C.

5. Procédé suivant l'une quelconque des revendications 1 à 4, caractérisé en ce qu'au moins deux lits d'absorbant sont employés et que, pendant qu'au moins un lit est en phase absorption, au moins un autre des lits est soumis à l'augmentation de température et ensuite, ce lit au moins qui a subi l'augmentation de température est remis en phase adsorption.

6. Procédé suivant l'une quelconque des revendications 1 à 5, caractérisé en ce que la charge d'alimentation est aussi traitée avec un tamis moléculaire et la régénération du tamis moléculaire est effectuée par chauffage, et que la régénération du tamis moléculaire est effectuée en même temps que l'augmentation temporaire de température du lit d'absorbant.

7. Procédé suivant la revendication 6, caractérisé en ce que le tamis moléculaire et le lit d'absorbant se trouvent dans le même récipient.
